

3,551,216

METHOD OF PRODUCING A STEEL PACKING  
STRIP OF HIGH STRENGTH

Herbert Severing, Hohenlimburg, Dieter Radtke, Letmathe, Hans-Wilhelm Grasshoff, Hagen, and Heinz Kress, Holzen, Germany, assignors to Hoesch Aktiengesellschaft Hauptverwaltung, Dortmund, Germany  
No Drawing. Filed Oct. 3, 1968, Ser. No. 764,955  
Claims priority, application Germany, Nov. 23, 1967,

1,608,163

Int. Cl. C21d 1/26

U.S. Cl. 148—12

5 Claims

## ABSTRACT OF THE DISCLOSURE

A steel packing strip with a tensile strength of around 95 to 125 kp./mm.<sup>2</sup>, an elongation  $\delta_5$  of 10 to 17% and a yield point ratio of 0.86 to 0.98 is produced from a hot rolled steel strip of a composition of about 0.35 to 0.80% C, 0.15 to 0.50% Si, possibly as much as 0.045% of P and S, 0.4% to 2% Mn and/or Ni, and the balance substantially all iron of sorbitic or intermediate stage structure after hot rolling to the desired thickness of about 0.30 to 1.30 mm. is cold rolled and is finally subjected to a continuous brief recovery annealing with the beginning of recrystallization at a temperature between about 500 and 680° C., Mn and/or Ni content decreasing with increase in the content of carbon.

## BACKGROUND OF THE INVENTION

## (1) Field of the invention

The invention relates to a process for producing a steel packing strip of high strength with a tensile strength of about 95 to 125 kp./mm.<sup>2</sup>, an elongation  $\delta_5$  of 10 to 17% and a yield point ratio of 0.86 to 0.98.

## (2) The prior art

It is known to produce packing strip with a tensile strength of less than 96 kp./mm.<sup>2</sup> by the relaxation and recovery annealing of cold rolled strip of a steel of the type of DIM 1624, as well as undoxidized, half-deoxidized or completely deoxidized structural steel with additives corresponding to DIN 17100 with the desired tensile strength value. The relaxation and recovery annealing can be carried out in continuous, pot or cupola annealing ovens. The high strength packing strip with a tensile strength of more than 95 kp./mm.<sup>2</sup> is produced in a known way through a continuous or intermittent heating in two heat treatments from a steel with a composition of about 0.20 to 0.40% C, 0.15 to 0.50%, Si, 1.0 to 1.5 Mn and, times, as much as 0.35% P and S.

A disadvantage of packing strips with a tensile strength of less than 95 kp./mm.<sup>2</sup> is that they require a quite large cross section and for the same reason also substantial weight, in order to have adequate packing characteristics. A further disadvantage in the production of packing strips with a tensile strength of more than 95 kp./mm.<sup>2</sup> is that two heat treatments are required, so that a yield point of only 0.75 to 0.85 is obtained.

## SUMMARY OF THE DISCLOSURE

The purpose of the present invention is to overcome these disadvantages in the known processes for the production of packing strips and to produce a packing strip which has a tensile strength of around 95 to 125 kp./mm.<sup>2</sup>, an elongation  $\delta_5$  of 10 to 17% and a yield point ratio of 0.86 to 0.98, which can be carried out in a simple manner with only one heat treatment.

This is achieved according to the invention by starting with a hot rolled strip with a composition of about 0.35 to 0.80% C.

0.15 to 0.50% Si

5 possibly 0.045% P and S

0.40 to 2.0% Mn and/or NiC

balance substantially all iron

of sorbitic or intermediate stage structure after the hot rolling to the desired thickness of around 0.30 to 1.30 mm. is cold rolled and finally subjected to a continuous brief recovery annealing with the beginning of recrystallization at temperatures of 500 to 680° C. In order to obtain the desired mechanical characteristics, advantageous

15ly the carbon content of the steel strip used is varied inversely with that of the manganese and/or nickel content. Because the carbon content influences strongly the working in hot and cold rolling, it is advantageous for the production of packing strip according to the invention

20 to use a steel strip with a carbon content of 0.40% and manganese or nickel of 1.5 to 2%. If a steel strip with a higher carbon content than 0.40% is used, then according to the invention the manganese and/or nickel content is correspondingly reduced. A further advantageous embodiment of the process according to the invention is to wind up the steel strip after the hot rolling at a reeling temperature of between 500 and 620° C.

The advantages achieved according to the process of the invention are especially that, for the production of a high yield point ratio of about 0.86 to 0.98 with a simultaneous elongation of 10 to 17% and a tensile strength of 95 kp./mm.<sup>2</sup>, only one heat treatment for a very short time and at a reduced temperature is necessary, and, in contrast to a packing strip with a tensile strength of less than 95 kp./mm.<sup>2</sup> and an elongation of 6 to 10%, the new packing strip can be more highly loaded, so as to save weight.

DESCRIPTION OF THE PREFERRED  
EMBODIMENTS

The following is an example of the process according to the invention.

A steel strip with a composition of:

45 0.47% C. 0.018% P  
0.21% Si 0.014% S  
1.43% Mn balance iron

is hot rolled to 1.50 mm. and is reeled at a temperature of about 560 to 580° C., so that for the subsequent cold rolling a sorbitic starting structure is obtained. Without difficulty (such as production of cracks in the edges of the strip) this hot strip is cold rolled to 0.5 or 0.8 mm. and finally in an annealing oven is subjected in the presence of a neutral protective gas at a temperature of 600° C. for two minutes to a recovery annealing (with a beginning of recrystallization). After this annealing treatment a finished packing strip with a full mechanical characteristic is measured:

| 60                   | Yield point<br>$\sigma_S$<br>kp./mm. <sup>2</sup> | Tensile strength<br>$\sigma_B$<br>kp./mm. <sup>2</sup> | Elongation<br>$\delta_5$ percent | Yield ratio,<br>$\sigma_S/\sigma_B$ |
|----------------------|---------------------------------------------------|--------------------------------------------------------|----------------------------------|-------------------------------------|
| Band thickness, mm.: |                                                   |                                                        |                                  |                                     |
| 0.50                 | 99.0                                              | 103.0                                                  | 15.0                             | 0.96                                |
| 0.80                 | 96.0                                              | 105.0                                                  | 14.5                             | 0.915                               |

65 While we have described here one embodiment of our invention, we wish it to be understood that we do not intend to limit ourselves thereby except within the scope of the claims hereto or hereinafter appended.

We claim:

70 1. Process for the production of steel packing strips with a tensile strength of about 95 to 125 kp./mm.<sup>2</sup>, elong-

gation  $\delta_5$  of 10 to 17%, and yield point ratio of 0.86 to 0.98, in which:

a hot rolled steel strip with a composition:

0.35 to 0.80% C

0.15 to 0.50% Si

0.40 to 2.0% of a metal selected from the group consisting of Mn and Ni  
balance essentially all iron

with a tensile strength of about 95 to 125 kp./mm.<sup>2</sup>, elongating to a thickness of about 0.30 to 1.50 mm. is cold rolled and thereafter subjected to a continuous brief recovery annealing with a beginning of recrystallization at temperature between 500 to 680° C., the content of said metal being substantially inversely proportional to the carbon content.

2. Process according to claim 1 in which said composition includes not more than 0.045% P and S.

3. Process according to claim 1 wherein the steel strip

after the hot rolling and before the cold rolling is reeled at a reel temperature of about 500 to 620° C.

4. Process according to claim 1 in which recovery annealing is carried out in an oven.

5. Process according to claim 1 wherein the recovery annealing is carried out in the presence of an inert protective gas.

#### References Cited

#### UNITED STATES PATENTS

|    |           |         |                |       |          |
|----|-----------|---------|----------------|-------|----------|
| 10 | 2,814,578 | 11/1957 | White          | ----- | 148—12   |
|    | 3,264,144 | 8/1966  | Frazier et al. | ----- | 148—12   |
|    | 3,311,512 | 3/1967  | Mohri et al.   | ----- | 148—12.1 |
|    | 3,421,951 | 1/1969  | Shelton        | ----- | 148—12.1 |

15 L. DEWAYNE RUTLEDGE, Primary Examiner

W. W. STALLARD, Assistant Examiner

U.S. CL. X.R.

20 148—12.1